

## UNITED STATES PATENT OFFICE.

ALFRED MILLER, OF DESSAU IN ANHALT, GERMANY, ASSIGNOR TO I. G. FARBEN-  
INDUSTRIE AKTIENGESELLSCHAFT, OF FRANKFORT-ON-THE-MAIN, GERMANY.

## METHOD OF MAKING PHOTOGRAPHIC COPIES BY REVERSAL.

No Drawing. Application filed September 23, 1925, Serial No. 58,191, and in Germany March 21, 1925.

The present invention relates to a method of making photographic copies of prints, drawings and the like by reversal.

In the art of making photographic copies of line drawings, printed text and the like, it was heretofore practically necessary to prepare a negative from which the positive could be printed.

Attempts have been made to produce positives directly, i. e. without first making negatives, but the methods in this direction have not been a practical success. As a general rule they are too tedious or too unreliable.

15 The object of the present invention is a simple and reliable method of directly making positives by reversal.

The invention is based upon the well-known hardening action of certain metallic salts upon the gelatines. If, for instance, a ferric chloride solution is allowed to act upon a negative produced upon a silver bromide gelatine, the solution penetrates those places which are free of silver and 20 effects a tanning action. However, at the places covered by a silver deposit, the ferric chloride penetrates comparatively slowly because of the reduction of ferric chloride to ferrous chloride as the result of the reaction 25 with the metallic silver which is re-converted to silver salt.

It was found that the difference between the relative rates of penetration may be increased by the addition of potassium ferricyanide, to the ferric chloride solution. To 30 facilitate the conversion of the metallic silver deposit into a silver salt some potassium bromide may be further added.

When a freshly developed and rinsed 35 negative produced upon a silver bromide gelatine plate is subjected, while being agitated as little as possible, to the action of the 40 solution just described, a well-known reaction takes place immediately at the places colored by the silver deposit resulting in a 45 superficial precipitate of Berlin blue, which for a brief period protects the underlying layer of gelatine against the penetration of the ferric chloride, whereas at the places 50 where there is no deposit of silver, the latter is free to penetrate and effect its tanning action.

When the superficially adhering Berlin blue is now washed off with cold water, it

can be observed that it readily adheres to 55 the places where there was no silver deposit or, in other words, where the emulsion was not exposed to light. The Berlin blue is apparently held by the tanning action and mordant action of the ferric chloride. At 60 any rate, the transfer of the Berlin blue away from the places where it was formed, i. e. the places where the silver was deposited, to the places where no silver was deposited, brings about a blue picture upon a 65 white back-ground. The original silver picture of the negative is bleached while the remaining part is coloured, which represents a total reversion of the picture. This silver salts formed by the reaction with the metallic silver deposit may be removed in well-known manner.

Since the Berlin blue spreading over the unexposed areas and deposited thereon is derived from the places where metallic silver was deposited, as described, it would be difficult to deposit a sufficient amount thereof on larger unexposed areas. This can be readily remedied by following up the ferric chloride-potassium ferricyanide bath with a 75 bath of potassium ferrocyanide of suitable degree of concentration, which causes at the unexposed places, where ferric chloride has penetrated into the layer of gelatine, the original formation of Berlin blue. At the 80 places originally containing a silver deposit and subsequently covered with a precipitate of Berlin blue the excess of ferric chloride, due to the action of the potassium ferrocyanide bath with the resulting formation of 85 fresh Berlin blue, is at once prevented from penetrating and hardening the underlying gelatine layer, whereby a subsequent hardening of these places, which might tend to affect the whiteness of the back-ground, is 90 precluded.

Best suited for carrying out the invention are unhardened emulsions of medium thickness and of steep gradation. By application of films or transparent paper the reproduced 100 print or drawing appears correct when viewed through the support or carrier. With an opaque support it is necessary to use an inverting prism or its equivalent to obtain lateral inversion of the image, as is well understood. As an alternative, the picture may be made in the manner described 105 and the support may be made transparent.

so that the picture may be viewed through it. The process may be carried out as follows:

5 The developed negative is well rinsed and then immersed for the period of about 20 seconds, while avoiding as much as possible movement thereof in the bath, in a solution containing approximately 1000 parts water, 100 parts potassium ferricyanide, 20 parts ferric chloride, 15 parts potassium bromide.

10 Then the negative is taken out and at once rinsed under a spray, then placed in a water bath and fixed and then again placed in water. Or, after the treatment with the solution, the negative may be placed into a 15 bath of a 25 per cent potassium ferrocyanide solution and then rinsed and fixed as before.

When the layer is sufficiently thin and the tanning action has reached the bottom the unhardened places may be washed off in 20 warm water, whereupon the tanned places, i. e. the areas representing the text of the lines of a drawing, may be specially treated with dyes or the like to accentuate the visible effect.

25 While in the foregoing reference was made to iron salts other salts may find application, for instance uranium salts, which have an analogous action.

To intensify the hardening effect there 30 may be added other compounds, such as formaldehyde or quinone. It is also sometimes desirable to use other metal salts, for instance uranium salts, in addition to the iron salts. The visible effect produced and 35 representing the original may be given a greater covering power by a suitable subsequent treatment. The blue picture hereinbefore referred to may be suitably toned, for instance by means of tannic acid. Also the 40 presence of dyes, especially mordant dyes, in the hardening or fixing bath act in the same manner.

I claim,

1. In a method of making photographic 45 reproductions, the step which consists in treating a freshly developed silver negative with an aqueous solution containing ferric chloride and potassium ferri-cyanide.

50 2. In a method of making photographic reproductions, the step which consists in treating a freshly developed silver negative with an aqueous solution containing ferric

chloride, potassium ferri-cyanide and potassium bromide.

3. In a method of making photographic 55 reproductions, the steps which consist in treating a freshly developed silver negative with an aqueous solution containing ferric chloride, potassium ferri-cyanide and potassium bromide, whereby a removable protective layer is formed by reaction with the 60 silver deposit at the places which have been exposed to light, and removing the said layer.

4. In a method of making photographic 65 reproductions the steps which consist in treating a freshly developed silver negative with an aqueous solution of ferric chloride and potassium ferricyanide, causing a tanning of the portions not covered by a silver 70 deposit and reacting with the silver deposit to form upon the portions covered thereby a loosely adhering layer of Berlin blue and rinsing the negative thus treated, thereby removing the Berlin blue from its places of 75 formation and spreading it over the tanned portions.

5. In a method of making photographic reproductions the steps which consist in treating a freshly developed silver negative 80 with an aqueous solution of ferric chloride, potassium ferricyanide and potassium bromide, rinsing the negative after treatment and subjecting it to the action of a potassium 85 ferrocyanide solution.

6. In a method of making photographic reproductions the step which consists in treating a freshly developed silver negative with a solution of about 100 parts of potassium ferricyanide, 20 parts ferric chloride 90 and 15 parts potassium bromide in about 1000 parts of water.

7. In a method of making photographic reproductions the steps which consist in 95 treating a freshly developed silver negative with a solution of about 100 parts potassium ferricyanide, 20 parts ferric chloride and 15 parts of potassium bromide in about 1000 parts of water and subsequently bathing the negative in an approximately 25 per cent solution of potassium ferrocyanide.

In testimony whereof, I affix my signature.

DR. ALFRED MILLER.